



US011492677B2

(12) **United States Patent**  
**Hasegawa et al.**

(10) **Patent No.:** **US 11,492,677 B2**  
(b4) **Date of Patent:** **Nov. 8, 2022**

(54) **HIGH-STRENGTH STEEL SHEET AND METHOD FOR PRODUCING THE SAME**

(71) Applicant: **JFE Steel Corporation**, Tokyo (JP)

(72) Inventors: **Hiroshi Hasegawa**, Tokyo (JP); **Hidekazu Minami**, Tokyo (JP); **Tatsuya Nakagaito**, Tokyo (JP); **Kana Sasaki**, Tokyo (JP); **Shoji Tanaka**, Tokyo (JP)

(73) Assignee: **JFE Steel Corporation**, Tokyo (JP)

(\*) Notice: Subject to any disclaimer, the term of this patent is extended or adjusted under 35 U.S.C. 154(b) by 376 days.

(21) Appl. No.: **16/957,739**

(22) PCT Filed: **Oct. 9, 2018**

(86) PCT No.: **PCT/JP2018/037569**

§ 371 (c)(1),

(2) Date: **Jun. 25, 2020**

(87) PCT Pub. No.: **WO2019/130713**

PCT Pub. Date: **Jul. 4, 2019**

(65) **Prior Publication Data**

US 2021/0062282 A1 Mar. 4, 2021

(30) **Foreign Application Priority Data**

Dec. 27, 2017 (JP) ..... JP2017-251048

(51) **Int. Cl.**

**C21D 9/46** (2006.01)  
**C21D 8/02** (2006.01)  
**C22C 38/00** (2006.01)  
**C22C 38/02** (2006.01)  
**C22C 38/04** (2006.01)  
**C22C 38/06** (2006.01)  
**C22C 38/42** (2006.01)  
**C22C 38/44** (2006.01)  
**C22C 38/46** (2006.01)  
**C22C 38/48** (2006.01)  
**C22C 38/50** (2006.01)  
**C22C 38/60** (2006.01)  
**C23C 2/40** (2006.01)

(52) **U.S. Cl.**

CPC ..... **C21D 9/46** (2013.01); **C21D 8/0226** (2013.01); **C21D 8/0236** (2013.01); **C21D 8/0273** (2013.01); **C22C 38/008** (2013.01); **C22C 38/02** (2013.01); **C22C 38/04** (2013.01); **C22C 38/06** (2013.01); **C22C 38/42** (2013.01); **C22C 38/44** (2013.01); **C22C 38/46** (2013.01); **C22C 38/48** (2013.01); **C22C 38/50** (2013.01); **C22C 38/60** (2013.01); **C23C 2/40** (2013.01); **C21D 2211/001** (2013.01); **C21D 2211/002** (2013.01); **C21D 2211/005** (2013.01); **C21D 2211/008** (2013.01)

(58) **Field of Classification Search**

CPC ..... C21D 9/46  
See application file for complete search history.

(56) **References Cited**

U.S. PATENT DOCUMENTS

|                 |         |                         |
|-----------------|---------|-------------------------|
| 10,370,737 B2   | 8/2019  | Hasegawa et al.         |
| 2010/0132848 A1 | 6/2010  | Ikeda et al.            |
| 2014/0234659 A1 | 8/2014  | Kawata et al.           |
| 2014/0251513 A1 | 9/2014  | Kami et al.             |
| 2016/0312329 A1 | 10/2016 | Hasegawa et al.         |
| 2017/0088914 A1 | 3/2017  | Ikeda et al.            |
| 2017/0260599 A1 | 9/2017  | Puerta Velasquez et al. |
| 2018/0002771 A1 | 1/2018  | Han et al.              |
| 2018/0010227 A1 | 1/2018  | Ikeda et al.            |
| 2018/0030565 A1 | 2/2018  | Hasegawa et al.         |
| 2018/0171459 A1 | 6/2018  | Drillet et al.          |
| 2019/0040511 A1 | 2/2019  | Hasegawa et al.         |

FOREIGN PATENT DOCUMENTS

|    |             |         |
|----|-------------|---------|
| CN | 103827341 A | 5/2014  |
| CN | 104245999 A | 12/2014 |
| CN | 104928579 A | 9/2015  |
| CN | 105531388 A | 4/2016  |
| CN | 106987790 A | 7/2017  |
| CN | 108603263 A | 9/2018  |
| CN | 110121568 A | 8/2019  |
| EP | 2762600 A1  | 8/2014  |

(Continued)

OTHER PUBLICATIONS

Korean Notice of Allowance for Korean Application No. 10-2020-7018283, dated Apr. 20, 2022, with translation, 4 pages.

Zhongzhi et al., "Electrical Steel", Beijing Metallurgical Industry Press, 2012, 4 pages.

Chinese Office Action for Chinese Application No. 201880084272.0, dated Apr. 6, 2021 with Concise Statement of Relevance of Office Action, 15 pages.

Korean Office Action for Korean Application No. 10-2020-7018283, dated Oct. 15, 2021, with Concise Statement of Relevance of Office Action, 7 pages.

Extended European Search Report for European Application No. 18895 022.4, dated Oct. 26, 2020, 14 pages.

(Continued)

Primary Examiner — Jophy S. Koshy

(74) Attorney, Agent, or Firm — RatnerPrestia

(57) **ABSTRACT**

A high-strength steel sheet has a specific composition and a microstructure. In the microstructure, the area fraction of elongated ferrite phase grains having an aspect ratio of 3 or more is 1% or less, the average crystal grain size of martensite included in a region extending 50  $\mu\text{m}$  from a surface of the steel sheet is 20  $\mu\text{m}$  or less, the content of oxide particles having a minor axis length of 0.8  $\mu\text{m}$  or less in the region extending 50  $\mu\text{m}$  from the surface of the steel sheet is  $1.0 \times 10^{10}$  particles/ $\text{m}^2$  or more, and the content of coarse oxide particles having a minor axis length of more than 1  $\mu\text{m}$  in the region extending 50  $\mu\text{m}$  from the surface of the steel sheet is  $1.0 \times 10^8$  particles/ $\text{m}^2$  or less. The content of hydrogen trapped in the steel sheet is 0.05 ppm by mass or more.

| (56) | <b>References Cited</b>  |         |    |               |         |
|------|--------------------------|---------|----|---------------|---------|
|      | FOREIGN PATENT DOCUMENTS |         | JP | 2015193907 A  | 11/2015 |
| EP   | 2762603 A1               | 8/2014  | JP | 2016128598 A  | 7/2016  |
| EP   | 2944705 A1               | 11/2015 | JP | 2017002384 A  | 1/2017  |
| EP   | 3040440 A1               | 7/2016  | JP | 2017048412 A  | 3/2017  |
| EP   | 3409807 A1               | 12/2018 | JP | 2018012884 A  | 1/2018  |
| EP   | 3421633 A1               | 1/2019  | JP | 2018521222 A  | 8/2018  |
| EP   | 3564400 A1               | 11/2019 | WO | 2013047760 A1 | 4/2013  |
| JP   | 2005063548 A             | 3/2005  | WO | 2015198582 A  | 12/2015 |
| JP   | 2009275266 A             | 11/2009 | WO | 2016098964 A1 | 6/2016  |
| JP   | 2010126787 A             | 6/2010  | WO | 2016113788 A1 | 7/2016  |
| JP   | 5402357 B2               | 1/2014  | WO | 2016129213 A1 | 8/2016  |
| JP   | 5633653 B1               | 12/2014 | WO | 2017131054 A1 | 8/2017  |
| JP   | 2013047812 A1            | 3/2015  | WO | 2017168962 A1 | 10/2017 |
| JP   | 5803836 B2               | 11/2015 |    |               |         |

OTHER PUBLICATIONS

International Search Report and Written Opinion for International Application No. PCT/JP2018/037569, dated Jan. 15, 2019, 6 pages.

## 1

**HIGH-STRENGTH STEEL SHEET AND METHOD FOR PRODUCING THE SAME****CROSS REFERENCE TO RELATED APPLICATIONS**

This is the U.S. National Phase application of PCT/JP2018/037569, filed Oct. 9, 2018, which claims priority to Japanese Patent Application No. 2017-251048 filed Dec. 27, 2017, the disclosures of these applications being incorporated herein by reference in their entireties for all purposes.

**FIELD OF THE INVENTION**

The present invention relates to a high-strength steel sheet excellent in terms of strength and workability and suitable for an automotive member and a method for producing the high-strength steel sheet.

**BACKGROUND OF THE INVENTION**

Steel sheets used for producing automotive components have been required to have high strengths in order to improve the collision safety and the fuel economy of automobiles. Since an increase in the strength of a steel sheet commonly leads to the degradation of the workability (bendability) of the steel sheet, the development of a steel sheet excellent in terms of strength and workability has been anticipated. While the application of high-strength steel sheets having a tensile strength (hereinafter, abbreviated as "TS") of more than 980 MPa has been increased recently, the high-strength steel sheets are typically worked into members, rocker components, and the like having a straight shape by primarily being bent because of great difficulty in forming the high-strength steel sheets into shape. Therefore, in such steel sheets, having excellent bendability have been anticipated. Accordingly, there have been various attempts to develop high-strength steel sheets having excellent bendability. For example, Patent Literature 1 discloses a technology in which a steel sheet having excellent bendability is produced by reducing the average crystal grain size of tempered-martensite. Patent Literature 2 discloses a technology in which a steel sheet having excellent bendability is produced by controlling the contents and shapes of inclusions and precipitates.

**PATENT LITERATURE**

PTL 1: International Publication No. 2016-113788  
PTL 2: International Publication No. 2015-198582

**SUMMARY OF THE INVENTION**

A high-strength steel sheet more excellent in both strength and workability than the related art, such as Patent Literature 1 and Patent Literature 2, and a method for producing the high-strength steel sheet are anticipated.

Aspects of the present invention were made to address the above issue. An object according to aspects of the present invention is to provide a high-strength steel sheet further excellent in both strength and workability and a method for producing the high-strength steel sheet.

In Patent Literature 1 and Patent Literature 2, attention is focused on only the microstructure of steel or the inclusions present in a steel sheet, and no discussion is made focusing on the hydrogen trapped in steel, that is, "trapped hydrogen".

## 2

The inventors of the present invention focused on the trapped hydrogen and made the present invention as described below.

The inventors of the present invention conducted extensive studies in order to achieve the above object and, as a result, found that the bendability of a steel sheet may be markedly enhanced when hydrogen is introduced into the steel sheet so as to be trapped by oxides and form trapped hydrogen while the microstructure of the steel sheet is optimized.

Specifically, a steel sheet may have a high strength and excellent bendability when the composition of the steel sheet is adjusted to be a specific composition; the microstructure of the steel sheet includes lower bainite, martensite, retained austenite, upper bainite, and ferrite such that the total area fraction of the lower bainite, the martensite, and the retained austenite is 40% to 100%, the area fraction of the retained austenite is 15% or less, and the total area fraction of the upper bainite and the ferrite is 0% to 60%; in the microstructure, the area fraction of elongated ferrite phase grains having an aspect ratio of 3 or more is adjusted to be 1% or less, the average crystal grain size of martensite included in a region extending 50  $\mu\text{m}$  from a surface of the steel sheet is adjusted to be 20  $\mu\text{m}$  or less, the content of oxide particles having a minor axis length of 0.8  $\mu\text{m}$  or less in the region extending 50  $\mu\text{m}$  from the surface of the steel sheet is adjusted to be  $1.0 \times 10^{10}$  particles/ $\text{m}^2$  or more, and the content of coarse oxide particles having a minor axis length of more than 1.0  $\mu\text{m}$  in the region extending 50  $\mu\text{m}$  from the surface of the steel sheet is adjusted to be  $1.0 \times 10^8$  particles/ $\text{m}^2$  or less; and the content of hydrogen trapped in the steel sheet is adjusted to be 0.05 ppm by mass or more.

In accordance with aspects of the present invention, the term "high strength" refers to the TS of the steel sheet being 980 MPa or more and being preferably 1180 MPa or more. The term "excellent bendability" used herein refers to the ratio (R/t) of the minimum bend radius R at which micro-cracks are absent to the thickness t of the steel sheet being 1.5 or less when the TS is 980 MPa or more and less than 1180 MPa, 2.5 or less when the TS is 1180 MPa or more and less than 1320 MPa, 3.5 or less when the TS is 1320 MPa or more and less than 1600 MPa, and 5.0 or less when the TS is 1600 MPa or more and less than 2100 MPa.

In accordance with aspects of the present invention, the term "microcracks" refers to cracks having a length of 0.5 mm or more.

Aspects of the present invention were made on the basis of the above findings. The summary of aspects of the present invention is as follows.

[1] A high-strength steel sheet including a composition containing, by mass, C: 0.05% to 0.40%, Si: 0.10% to 3.0%, Mn: 1.5% to 4.0%, P: 0.100% or less (excluding 0%), S: 0.02% or less (excluding 0%), Al: 0.010% to 1.0%, and N: 0.010% or less, with the balance being Fe and inevitable impurities; a microstructure including lower bainite, martensite, retained austenite, upper bainite, and ferrite such that the total area fraction of the lower bainite, the martensite, and the retained austenite is 40% to 100%, the area fraction of the retained austenite is 15% or less, and the total area fraction of the upper bainite and the ferrite is 0% to 60%, wherein, in the microstructure, the area fraction of elongated ferrite phase grains having an aspect ratio of 3 or more is 1% or less, the average crystal grain size of martensite included in a region extending 50  $\mu\text{m}$  from a surface of the steel sheet is 20  $\mu\text{m}$  or less, the content of oxide particles having a minor axis length of 0.8  $\mu\text{m}$  or less in the region extending 50  $\mu\text{m}$  from the surface of the steel sheet is  $1.0 \times 10^{10}$

particles/m<sup>2</sup> or more, and the content of coarse oxide particles having a minor axis length of more than 1.0 µm in the region extending 50 µm from the surface of the steel sheet is 1.0×10<sup>8</sup> particles/m<sup>2</sup> or less; and a content of hydrogen trapped in the steel sheet is 0.05 ppm by mass or more.

[2] The high-strength steel sheet described in [1], further including one or more elements selected from, by mass, Cr: 0.005% to 2.0%, Ti: 0.005% to 0.20%, Nb: 0.005% to 0.20%, Mo: 0.005% to 2.0%, V: 0.005% to 2.0%, Ni: 0.005% to 2.0%, Cu: 0.005% to 2.0%, B: 0.0001% to 0.0050%, Ca: 0.0001% to 0.0050%, REM: 0.0001% to 0.0050%, Sn: 0.01% to 0.50%, and Sb: 0.0010% to 0.10%.

[3] The high-strength steel sheet described in [1] or [2], including a coating film constituted by one or more layers, the coating film being disposed on the surface of the steel sheet.

[4] The high-strength steel sheet described in [1] or [2], including a galvanizing layer disposed on the surface of the steel sheet.

[5] The high-strength steel sheet described in [1] or [2], including an alloyed hot-dip galvanizing layer disposed on the surface of the steel sheet.

[6] A method for producing a high-strength steel sheet, the method including a hot-rolling step of rough-rolling a slab having the composition described in [1] or [2], subsequently performing descaling at a pressure of 15 MPa or more, then performing finish rolling at 800°C. to 950°C., performing cooling subsequent to the finish rolling, and then performing coiling at 550°C. or less; an annealing step of heating a hot-rolled steel sheet produced in the hot-rolling step to 730°C. to 950°C. and performing holding at 730°C. to 950°C. in an atmosphere having a hydrogen concentration of 1.0% to 35.0% by volume and a dew point of -35°C. to 15°C. for 10 to 1000 s; a cooling step of cooling a steel sheet treated in the annealing step to 600°C. at an average rate of 5°C./s or more, stopping the cooling at a temperature of more than Ms and 600°C. or less, subsequently performing retention at a temperature of more than Ms and 600°C. or less for 1000 s or less, and, subsequent to the retention, performing cooling to room temperature such that the average cooling rate between Ms and 50°C. is 1°C./s or more; an elongation rolling step of rolling a steel sheet treated in the cooling step at an elongation ratio of 0.05% to 1%; and an aging treatment step of subjecting a steel sheet treated in the elongation rolling step to an aging treatment under conditions satisfying Formula (1) below,

$$(273+T) \times (20+\log_{10}(t)) \geq 6800, \quad (1)$$

where T is a temperature (°C.) of 200°C. or less, and t is a time (hr).

[7] A method for producing a high-strength steel sheet, the method including a hot-rolling step of rough-rolling a slab having the composition described in [1] or [2], subsequently performing descaling at a pressure of 15 MPa or more, then performing finish rolling at 800°C. to 950°C., performing cooling subsequent to the finish rolling, and then performing coiling at 550°C. or less; a cold-rolling step of cold-rolling a hot-rolled steel sheet produced in the hot-rolling step at a rolling reduction ratio of 20% or more; an annealing step of heating a cold-rolled steel sheet produced in the cold-rolling step to 730°C. to 950°C. and performing holding at 730°C. to 950°C. in an atmosphere having a hydrogen concentration of 1% to 35% by volume and a dew point of -35°C. to 15°C. for 10 to 1000 s; a cooling step of cooling a steel sheet treated in the annealing step to 600°C. at an average rate of 5°C./s or more, stopping the cooling at a temperature of more than Ms and 600°C. or less, subsequently performing

ing retention at a temperature of more than Ms and 600°C. or less for 1000 s or less, and, subsequent to the retention, performing cooling to room temperature such that the average cooling rate between Ms and 50°C. is 1°C./s or more; an elongation rolling step of rolling a steel sheet treated in the cooling step at an elongation ratio of 0.05% to 1%; and an aging treatment step of subjecting a steel sheet treated in the elongation rolling step to an aging treatment under conditions satisfying Formula (1) below,

$$(273+T) \times (20+\log_{10}(t)) \geq 6800, \quad (1)$$

where T is a temperature (°C.) of 200°C. or less, and t is a time (hr).

[8] The method for producing a high-strength steel sheet described in [6] or [7], wherein a coating film formation treatment is performed in any of the steps subsequent to the annealing step.

[9] The method for producing a high-strength steel sheet described in [6] or [7], wherein a galvanizing treatment is performed in the cooling step.

[10] The method for producing a high-strength steel sheet described in [9], wherein an alloying treatment is further performed subsequent to the galvanizing treatment.

According to aspects of the present invention, a high-strength steel sheet having excellent bendability can be produced. The high-strength steel sheet can be suitable as a material for automotive components.

#### DETAILED DESCRIPTION OF EMBODIMENTS OF THE INVENTION

An embodiment of the present invention is described below. The present invention is not limited to the embodiment below.

Firstly, the composition of the high-strength steel sheet according to aspects of the present invention is described below. In the following description, “%” used for describing the content of an element means “% by mass” unless otherwise specified. In accordance with aspects of the present invention, “to” means that the values described before and after “to” are included as the lower and upper limits, respectively.

C: 0.05% to 0.40%

C is an element that causes the formation of martensite, bainite, and the like and thereby effectively increases the TS of the steel sheet. If the C content is less than 0.05%, the above advantageous effects may fail to be achieved sufficiently and, consequently, a TS of 980 MPa or more may fail to be achieved. Accordingly, the C content is limited to be 0.05% or more. The C content is preferably 0.07% or more, is more preferably 0.09% or more, and is still more preferably 0.11% or more. If the C content exceeds 0.40%, hardening of martensite may occur, which may significantly degrade the bendability of the steel sheet. Accordingly, the

C content is limited to be 0.40% or less. The C content is preferably 0.37% or less, is more preferably 0.35% or less, and is further preferably 0.32% or less.

Si: 0.10% to 3.0%

Si is an element that causes the solid-solution strengthening of steel and thereby effectively increases the TS of the steel sheet. In addition, oxides including Si are effective in trapping hydrogen. In order to achieve the advantageous effect of oxides including Si, the Si content is limited to be 0.10% or more. The Si content is preferably 0.20% or more, is more preferably 0.30% or more, and is further preferably 0.40% or more. If the Si content exceeds 3.0%, steel may become brittle and the bendability of the steel sheet may

become significantly degraded. Accordingly, the Si content is limited to be 3.0% or less. The Si content is preferably 2.5% or less, is more preferably 2.0% or less, and is further preferably 1.8% or less.

Min: 1.5% to 4.0%

Mn is an element that causes the formation of martensite, bainite, and the like and thereby effectively increases the TS of the steel sheet. If the Mn content is less than 1.5%, the above advantageous effects may fail to be achieved sufficiently and, consequently, a TS of 980 MPa or more may fail to be achieved. Accordingly, the Mn content is limited to be 1.5% or more. The Mn content is preferably 1.8% or more, is more preferably 2.0% or more, and is further preferably 2.2% or more. If the Mn content exceeds 4.0%, steel may become brittle and the bendability required in accordance with aspects of the present invention may fail to be achieved. Accordingly, the Mn content is limited to be 4.0% or less. The Mn content is preferably 3.8% or less, is more preferably 3.6% or less, and is further preferably 3.4% or less.

P: 0.100% or Less (Excluding 0%)

Since P causes grain boundary embrittlement and thereby degrades the bendability of the steel sheet, it is desirable to reduce the P content to a minimum level. The P content allowable in accordance with aspects of the present invention is 0.100% or less. The P content is preferably 0.050% or less. Although the lower limit is not specified, the P content is preferably 0.001% or more in consideration of production efficiency, because production efficiency may be reduced if the P content is less than 0.001%.

S: 0.02% or Less (Excluding 0%)

Since S causes an increase in the content of inclusions and thereby degrades the bendability of the steel sheet, it is preferable to reduce the S content to a minimum level. The S content allowable in accordance with aspects of the present invention is 0.02% or less. The S content is preferably 0.01% or less. Although the lower limit is not specified, the S content is preferably 0.0005% or more in consideration of production efficiency, because production efficiency may be reduced if the S content is less than 0.0005%.

Al: 0.010% to 1.0%

Al serves as a deoxidizing agent and is preferably added to steel in a deoxidation process. Accordingly, the Al content is limited to be 0.010% or more. The Al content is preferably 0.015% or more. If the Al content is excessively high, a large amount of soft ferrite phase may be formed, which results in a reduction in TS. The Al content allowable in accordance with aspects of the present invention is 1.0% or less. The Al content is preferably 0.50% or less.

N: 0.010% or Less

If the N content exceeds 0.010%, coarse nitride particles may be formed, which results in the degradation of bendability. Accordingly, the N content is limited to be 0.010% or less. Although the lower limit is not specified, the N content is preferably 0.0005% or more in consideration of production efficiency, because production efficiency may be reduced if the N content is less than 0.0005%.

The composition according to aspects of the present invention may contain the elements described below as optional constituents.

Cr: 0.005% to 2.0%, Ti: 0.005% to 0.20%, Nb: 0.005% to 0.20%, Mo: 0.005% to 2.0%, V: 0.005% to 2.0%, Ni: 0.005% to 2.0%, Cu: 0.005% to 2.0%, B: 0.0001% to 0.0050%, Ca: 0.0001% to 0.0050%, REM: 0.0001% to 0.0050%, Sn: 0.01% to 0.50%, and Sb: 0.0010% to 0.10%

Cr, Cu, and Ni are elements that cause the formation of martensite and bainite and thereby effectively increase the strength of the steel sheet. In order to achieve the above

advantageous effects, the contents of Cr, Cu, and Ni are preferably 0.005% or more. The contents of Cr, Cu, and Ni are more preferably 0.010% or more and are further preferably 0.050% or more. If the content of Cr, Cu, or Ni exceeds 2.0%, a large amount of retained austenite may remain in steel and, consequently, the bendability of the steel sheet may become slightly degraded. Accordingly, the contents of Cr, Cu, and Ni are preferably 2.0% or less. The contents of Cr, Cu, and Ni are more preferably 1.5% or less and are further preferably 1.0% or less.

Ti, Nb, V, and Mo are elements that cause the formation of carbides and thereby effectively increase the strength of the steel sheet. In order to achieve the above advantageous effects, the contents of Ti, Nb, V, and Mo are preferably 0.005% or more and are more preferably 0.010% or more. If the content of Ti, Nb, V, or Mo exceeds its upper limit, carbide particles may coarsen and the content of dissolved carbon may be reduced, which results in a reduction in the hardness of steel. Accordingly, the Ti content is preferably 0.20% or less, is more preferably 0.10% or less, and is further preferably 0.05% or less. The Nb content is preferably 0.20% or less, is more preferably 0.10% or less, and is further preferably 0.05% or less. The V content is preferably 2.0% or less, is more preferably 1.0% or less, and is further preferably 0.5% or less. The Mo content is preferably 2.0% or less, is more preferably 1.0% or less, and is further preferably 0.5% or less.

B is an element that enhances the hardenability of the steel sheet, causes the formation of martensite and bainite, and thereby effectively increases the strength of the steel sheet. In order to achieve the above advantageous effects, the B content is preferably 0.0001% or more and is more preferably 0.0005% or more. If the B content exceeds 0.0050%, the amount of inclusions may be increased and, consequently, the bendability of the steel sheet may become slightly degraded. Accordingly, the B content is preferably 0.0050% or less and is more preferably 0.0030% or less.

Ca and REM are elements that effectively enhance the bendability of the steel sheet by controlling the shapes of inclusions. In order to achieve the above advantageous effect, the contents of Ca and REM are preferably 0.0001% or more and are more preferably 0.0005% or more. If the content of Ca or REM exceeds 0.0050%, the amount of inclusions may be increased and, consequently, the bendability of the steel sheet may become slightly degraded. Accordingly, the contents of Ca and REM are preferably 0.0050% or less and are more preferably 0.0030% or less.

Sn and Sb are elements that effectively limit a reduction in the strength of steel by reducing decarburization, denitrification, boron removal, and the like. In order to achieve the above advantageous effects, the Sn content is preferably 0.01% or more or the Sb content is preferably 0.0010% or more. If the content of Sn or Sb exceeds its upper limit, grain boundary embrittlement may occur, which slightly degrades the bendability of the steel sheet. Accordingly, the Sn content is preferably 0.50% or less and is more preferably 0.10% or less. The Sb content is preferably 0.10% or less and is more preferably 0.05% or less.

The balance includes Fe and inevitable impurities. When the content of any of the above optional constituents is less than its lower limit, it is considered that the optional constituent serves as an inevitable impurity. The composition according to aspects of the present invention may optionally contain Zr, Mg, La, Ce, Bi, W, and Pb as inevitable impurities such that the total content of Zr, Mg, La, Ce, Bi, W, and Pb is 0.002% or less.

Total Area Fraction of Lower Bainite, Martensite, and Retained Austenite: 40% to 100%

If the total area fraction of lower bainite, martensite, and retained austenite is less than 40%, a TS of 980 MPa or more may fail to be achieved. Accordingly, the above total area fraction is limited to be 40% to 100%, is preferably 45% to 100%, and is more preferably 50% to 100%. The term "martensite" used herein refers to both as-quenched martensite and tempered martensite. The term "lower bainite" used herein refers to bainite that includes uniformly aligned carbide particles. Lower bainite may include tempered bainite.

The area fraction of martensite in the overall microstructure is preferably 30% or more and is more preferably 35% or more. The upper limit for the area fraction of martensite is preferably 99% or less, is more preferably 97% or less, and is further preferably 95% or less.

Area Fraction of Retained Austenite: 15% or Less

Retained austenite may transform into martensite in a bending work to promote the formation of cracks. The adverse effect becomes significant if the area fraction of retained austenite in the overall microstructure exceeds 15%. Accordingly, the area fraction of retained austenite is limited to be 15% or less, is preferably 10% or less, and is more preferably 8% or less. Although the lower limit for the area fraction of retained austenite is not specified and the area fraction of retained austenite may be 0%, the area fraction of retained austenite is preferably 1% or more and is more preferably 2% or more.

Total Area Fraction of Upper Bainite and Ferrite: 0% to 60%

If the total area fraction of upper bainite and ferrite exceeds 60%, a TS of 980 MPa or more may fail to be achieved. Accordingly, the total area fraction of upper bainite and ferrite is limited to be 0% to 60%, is preferably 0% to 50%, and is more preferably 0% to 45%. In particular, as for high-strength steel, the smaller the total area fraction of upper bainite and ferrite, the more preferable the steel sheet in terms of bendability. The above total area fraction is preferably 10% or less when the TS is 1320 MPa or more and less than 1600 MPa. The above total area fraction is preferably 3% or less when the TS is 1600 MPa or more and less than 2100 MPa. The term "upper bainite" used herein refers to bainite that does not include uniformly aligned carbide particles.

Area Fraction of Elongated Ferrite Phase Grains Having Aspect Ratio of 3 or More: 1% or Less

Elongated ferrite phase grains having a high aspect ratio may promote occurrence of cracking in a bending work and degrade the bendability of the steel sheet. In order to inhibit the adverse effects, it is necessary to limit the area fraction of elongated ferrite phase grains having an aspect ratio of 3 or more in the overall microstructure to be 1% or less. Accordingly, the area fraction of elongated ferrite phase grains having an aspect ratio of 3 or more is limited to be 1% or less.

Other Microstructure Components

The microstructure according to aspects of the present invention may include other microstructure components than the above described ones such that the total area fraction of the other microstructure components is 5% or less. Examples of the other microstructure components include pearlite.

Average Crystal Grain Size of Martensite Included in Region Extending 50 µm from Surface of Steel Sheet: 20 µm or Less

The region in which microcracks are formed in a bending work is primarily the region extending 50 µm from the

surface of the steel sheet (hereinafter, this region may be referred to as "surface layer" or "surface layer of the steel sheet"). When the average crystal grain size of martensite included in the region extending 50 µm from the surface of the steel sheet is 20 µm or less, the formation of microcracks in a bending work may be reduced and the bendability required in accordance with aspects of the present invention may be achieved. Accordingly, the average crystal grain size of martensite included in the region extending 50 µm from the surface of the steel sheet is limited to be 20 µm or less. Although the lower limit is not specified, the above average crystal grain size is commonly 1 µm or more.

In accordance with aspects of the present invention, the oxide particles dispersed in the surface layer of the steel sheet and the trapped hydrogen play an important role, and excellent bendability may be achieved when the above factors are controlled to fall within predetermined ranges. Although the mechanisms for this are not clarified, it is considered that, for example, when hydrogen is trapped by oxide particles included in the surface layer of the steel sheet, microvoids are likely to be formed in a bending work as a result of separation between the oxide particles and the base iron, which may cause plastic relaxation and reduce the formation of macro cracks.

Oxide Particles Having Minor Axis Length of 0.8 µm or Less in Region Extending 50 µm from Surface of Steel Sheet:  $1.0 \times 10^{10}$  Particles/m<sup>2</sup> or More Coarse Oxide Particles Having Minor Axis Length of More Than 1.0 µm in Region Extending 50 µm from Surface of Steel Sheet:  $1.0 \times 10^8$  Particles/m<sup>2</sup> or Less

If the content of oxide particles having a minor axis length of 0.8 µm or less in the region extending 50 µm from the surface of the steel sheet is less than  $1.0 \times 10^{10}$  particles/m<sup>2</sup>, the bendability required in accordance with aspects of the present invention may fail to be achieved. If the content of oxide particles having a minor axis length of more than 1.0 µm in the above region is more than  $1.0 \times 10^8$  particles/m<sup>2</sup>, the bendability of the steel sheet may become degraded.

Accordingly, the content of the oxide particles in the region extending 50 µm from the surface of the steel sheet is limited to be  $1.0 \times 10^{10}$  particles/m<sup>2</sup> or more and is preferably  $100.0 \times 10^{10}$  particles/m<sup>2</sup> or more. The content of oxide particles having a minor axis length of more than 1.0 µm is limited to be  $1.0 \times 10^8$  particles/m<sup>2</sup> or less and is more preferably  $1.0 \times 10^7$  particles/m<sup>2</sup> or less.

In the case where a coating film is present on the surface of the steel sheet, the interface between the base iron and the coating film is considered as the surface of the steel sheet. In accordance with aspects of the present invention, the term "oxide" refers primarily to a simple or complex oxide of Fe, Si, Mn, Al, Mg, Ti, or the like. The upper limit is not specified and is commonly  $500.0 \times 10^{10}$  particles/m<sup>2</sup> or less. Oxide particles having a minor axis length of more than 0.8 µm and less than 1.0 µm which are included in the region extending 50 µm from the surface of the steel sheet do not greatly affect the advantageous effects according to aspects of the present invention.

Hydrogen Trapped in Steel Sheet: 0.05 ppm by Mass or More

If the content of hydrogen trapped in the steel sheet is less than 0.05 ppm by mass, the bendability required in accordance with aspects of the present invention may fail to be achieved. Accordingly, the content of hydrogen trapped in the steel sheet is limited to be 0.05 ppm by mass or more and is preferably 0.07 ppm by mass or more. In accordance with aspects of the present invention, the term "trapped hydrogen" refers to hydrogen that is desorbed at 350° C. or more when thermal desorption is performed in the increasing

temperature at 200° C./hr. It is particularly preferable to limit the content of hydrogen that desorbs at 350° C. to 600° C. to be 0.05 ppm by mass or more. It is more preferable to limit the content of hydrogen that desorbs at 450° C. to 600° C. to be 0.05 ppm by mass or more. Although the upper limit is not specified, the content of hydrogen trapped in the steel sheet is commonly 1.00 ppm by mass or less. It is necessary to limit the content of hydrogen trapped in the steel sheet to be 0.05 ppm by mass or more prior to a bending work. However, even in a product that has been subjected to a bending work, when the content of hydrogen trapped in the steel sheet which is measured at an unbent portion of the steel sheet is 0.05 ppm by mass or more, it is considered that the content of hydrogen trapped in the steel sheet at the bent portion of steel sheet was 0.05 ppm by mass or more.

In accordance with aspects of the present invention, the area fraction of a microstructure component is the ratio of the area of the microstructure component to the area of observation. The area fractions of microstructure components are determined by taking a sample from an annealed steel sheet, grinding and polishing a cross section of the sample, the cross section being taken in the thickness direction of the steel sheet so as to be parallel to the rolling direction, performing etching with 3% nital, capturing an image of the cross section in the vicinity of the surface and at a position 300  $\mu\text{m}$  from the surface in the thickness direction with a SEM (scanning electron microscope) at 1500-fold magnification in 3 fields of view for each position, calculating the area fractions of the microstructure components with Image-Pro produced by Media Cybernetics, Inc. on the basis of the image data, and calculating the average of the area fractions of each of the microstructure components in the fields of view as the area fraction of the microstructure component. In the image data, ferrite is identified as black that does not contain carbides; upper bainite is identified as gray or dark gray that does not contain uniformly aligned carbide particles; retained austenite is identified as white or light gray; lower bainite is identified as gray or dark gray that contains uniformly aligned carbide particles; martensite is identified as white, or light gray, gray, or dark gray that contains carbides having a plurality of orientations; and pearlite is identified as a black and white lamellar microstructure. Carbide is identified as a dot-like or linear white microstructure. Note that, in accordance with aspects of the present invention, although plural types of martensite having different properties may exist depending on the tempering conditions as described above, the plural types of martensite formed under different tempering conditions are not distinguished from one another and collectively considered as martensite.

Since ferrite can be identified as black that does not contain carbides as described above, the area fraction of elongated ferrite phase grains having an aspect ratio of 3 or more can be determined from the above image data.

The area fraction of retained austenite phase can be determined by grinding the steel sheet that has been subjected to the final production step to a position  $\frac{1}{4}$  the thickness of the steel sheet, further polishing the resulting cross section by 0.1 mm by chemical polishing, measuring the integrated diffraction intensities on the (200), (220), and (311) planes of fcc iron (austenite phase) and the (200) plane, the (211) plane, and the (220) plane of bcc iron (ferrite phase) with an X-ray diffraction apparatus using Mo-K $\alpha$  radiation, and determining the volume fraction of retained austenite phase on the basis of the ratio of the integrated diffraction intensities measured on the above planes of fcc iron (austenite phase) to the integrated diffrac-

tion intensities measured on the above planes of bcc iron (ferrite phase). The above volume fraction is used as the area fraction of retained austenite phase. In accordance with aspects of the present invention, the area fraction of retained austenite phase was determined by the above-described method in which X-ray diffraction is used.

As for the oxide included in the surface layer of the steel sheet, the above sample is etched with 0.05% nital, an image of a region which extends 50  $\mu\text{m}$  from the surface layer of the steel sheet is captured with a SEM at 5000-fold magnification in 10 fields of view on a random basis, and the number of oxide particles having a minor axis length of 0.8  $\mu\text{m}$  or less and whether oxide particles having a minor axis length of more than 0.8  $\mu\text{m}$  are present are determined with Image-Pro produced by Media Cybernetics, Inc. on the basis of the image data. In the image data, oxide particles can be identified as dot-like or linear white portions. The average crystal grain size of martensite included in the surface layer of the steel sheet is also calculated using the above image data of the surface layer. Specifically, the average crystal grain size of martensite is determined by calculating the areas of martensite grains from the image data, calculating the equivalent circle diameters from the above areas as the crystal grain sizes of the martensite grains, and taking the number-average thereof. In the calculation of the average crystal grain size of martensite, the grain boundaries of martensite include the boundaries between martensite grains and prior-austenite grains or grains of other microstructure components and do not include packet boundaries and block boundaries.

The high-strength steel sheet according to aspects of the present invention that has the above-described composition, the above-described microstructure, etc. has a tensile strength (TS) of 980 MPa or more. Although the upper limit for the TS is not specified, the TS is preferably 2200 MPa or less in consideration of the balance between the TS and the other properties. The method for measuring the TS is as described in Examples below, that is, a method in which a JIS No. 5 tensile test specimen (JIS Z 2201) is taken from the steel sheet in a direction perpendicular to the rolling direction and the specimen is subjected to a tensile test conforming to JIS Z 2241 (1998) with a strain rate of  $10^{-3}/\text{s}$ .

The high-strength steel sheet according to aspects of the present invention has excellent bendability. Specifically, the ratio (R/t) of the minimum bend radius R determined by the following method to the thickness t of the steel sheet is 1.5 or less when the TS is 980 MPa or more and less than 1180 MPa, 2.5 or less when the TS is 1180 MPa or more and less than 1320 MPa, 3.5 or less when the TS is 1320 MPa or more and less than 1600 MPa, and 5.0 or less when the TS is 1600 MPa or more and less than 2100 MPa.

(Method for Measuring Bend Radius)

A strip-shaped test specimen having a width of 30 mm and a length of 100 mm is taken from the steel sheet such that the axis about which a bend test is conducted is parallel to the rolling direction. This specimen is subjected to a bend test. Specifically, the test specimen is subjected to a 90°-V bend test with a stroke speed of 50 mm/s, a pressing load of 10 ton, and a press holding time of 5 seconds. The ridge line formed at the vertex of the bent portion is observed with a 10-fold magnifier. The minimum one of bend radius at which cracks having a length of 0.5 mm or more are not formed is determined.

The high-strength steel sheet according to aspects of the present invention may include a coating film constituted by one or more layers which is disposed on the surface. Examples of the coating film include an organic coating

## 11

film, an inorganic coating film, and an inorganic-organic composite coating film. When the high-strength steel sheet includes the coating film, corrosion resistance, a rust prevention property, resistance to delayed fracture, design, lubricity, an antibacterial property, and the like may be enhanced.

The high-strength steel sheet according to aspects of the present invention may include a coated layer disposed on the surface. Examples of the coated layer include a hot-dip galvanizing layer, an electrogalvanizing layer, and a hot-dip aluminizing layer. The coated layer may be an alloyed hot-dip galvanizing layer produced by performing an alloying treatment subsequent to hot-dip galvanizing.

## Production Method

A method for producing the high-strength steel sheet according to aspects of the present invention includes a hot-rolling step of heating a slab having the above-described composition, rough-rolling the slab, subsequently performing descaling at a pressure of 15 MPa or more, then performing finish rolling at 800° C. to 950° C., performing cooling subsequent to the finish rolling, and then performing coiling at 550° C. or less to produce a hot-rolled steel sheet, an optional cold-rolling step of cold-rolling the hot-rolled steel sheet at a rolling reduction ratio of 20% or more to produce a cold-rolled steel sheet, an annealing step of heating the hot-rolled steel sheet or the cold-rolled steel sheet to 730° C. to 950° C. and performing holding at 730° C. to 950° C. in an atmosphere having a hydrogen concentration of 1.0% to 35.0% by volume and a dew point of -35° C. to 15° C. for 10 to 1000 s, a cooling step of cooling the annealed steel sheet to 600° C. at an average rate of 5° C./s or more, stopping the cooling at a temperature of more than Ms and 600° C. or less, subsequently performing retention at a temperature of more than Ms and 600° C. or less for 1000 s or less, and then performing cooling to room temperature such that the average cooling rate between Ms and 50° C. is 1.0° C./s or more, an elongation rolling step of rolling the steel sheet at an elongation ratio of 0.05% to 1%, and an aging treatment step of subjecting the steel sheet to an aging treatment under conditions satisfying the formula below.

$$(273+T) \times (20 + \log_{10}(t)) \geq 6800, T \leq 200,$$

where T is a temperature (° C.) and t is a time (hr).

## Descaling Pressure: 15 MPa or More

If the descaling pressure is less than 15 MPa, scales may remain on the steel sheet and increase the likelihood of coarse oxide particles being formed in the surface layer of the steel sheet by feeding oxygen while cooling is performed subsequent to coiling. This results in degradation of bendability. Accordingly, the descaling pressure is limited to be 15 MPa or more. Although the upper limit is not specified, the descaling pressure is preferably 75 MPa or less.

## Finish-Rolling Temperature: 800° C. to 950° C.

If the finish-rolling temperature is less than 800° C., ferrite may be formed and elongated ferrite grains may be formed in the surface layer of the hot-rolled steel sheet. The ferrite grains remain in the surface layer even after annealing to form elongated ferrite grains having an aspect ratio of 3 or more, which degrade the bendability of the steel sheet. If the finish-rolling temperature is more than 950° C., the average grain size of martensite included in the surface layer may be increased, which degrades the bendability of the steel sheet. Accordingly, the finish-rolling temperature is limited to be 800° C. to 950° C. As for the lower limit, the

## 12

finish-rolling temperature is preferably 830° C. or more. As for the upper limit, the finish-rolling temperature is preferably 920° C. or less.

## Coiling Temperature: 550° C. or Less

- 5 If the coiling temperature is more than 550° C., oxide particles having a minor axis length of more than 0.8 μm may be formed in the surface layer of the steel sheet and, consequently, the bendability required in accordance with aspects of the present invention may fail to be achieved.
- 10 Accordingly, the coiling temperature is limited to be 550° C. or less and is preferably 500° C. or less. Although the lower limit is not specified, the coiling temperature is preferably 250° C. or more in consideration of shape stability and the like.

## 15 Cold Rolling Reduction Ratio: 20% or More

- Cold rolling is not necessarily performed. When cold rolling is performed in accordance with aspects of the present invention, the rolling reduction ratio needs to be 20% or more. If the rolling reduction ratio is less than 20%, 20 coarse elongated ferrite grains may be formed during annealing, which results in the degradation of bendability. Accordingly, when cold rolling is performed, the rolling reduction ratio is limited to be 20% or more and is preferably 30% or more. Although the upper limit is not specified, the 25 rolling reduction ratio is preferably 90% or less in consideration of shape stability and the like.

## Annealing Temperature: 730° C. to 950° C.

- In the case where cold rolling is not performed, the hot-rolled steel sheet is annealed. In the case where cold 30 rolling is performed, the cold-rolled steel sheet is annealed. If the annealing temperature is less than 730° C., the formation of austenite may become insufficient. Since austenite formed by annealing is converted into martensite or bainite in the final microstructure by bainite transformation or martensite transformation, insufficient formation of austenite results in failure to achieve the intended microstructure. If the annealing temperature exceeds 950° C., coarse 35 grains may be formed. In such a case, the intended microstructure may also fail to be achieved. Accordingly, the annealing temperature is limited to be 730° C. to 950° C. As for the lower limit, the annealing temperature is preferably 750° C. or more. As for the upper limit, the annealing temperature is preferably 930° C. or less.

## Annealing Holding Time: 10 to 1000 s

- 40 If the annealing holding time is less than 10 s, the formation of austenite may become insufficient and, consequently, the intended microstructure or the intended amount of trapped hydrogen may fail to be achieved. If the annealing holding time exceeds 1000 s, coarse grains may be formed and, consequently, the intended microstructure according to aspects of the present invention may fail to be achieved. Accordingly, the annealing holding time is limited to be 10 to 1000 s. As for the lower limit, the annealing holding time is preferably 30 s or more. As for the upper limit, the 45 annealing holding time is preferably 500 s or less. In accordance with aspects of the present invention, the term "annealing holding time" refers to the amount of time during which the steel sheet is retained in an annealing temperature range described above. The temperature is not necessarily 50 maintained to be constant; the temperature may be increased or reduced within a range of 730° C. to 950° C.

## 55 Hydrogen Concentration in Atmosphere at 730° C. to 950° C.: 1.0% to 35.0% by Volume

- If the hydrogen concentration in the atmosphere at 730° 60 C. to 950° C. is less than 1.0% by volume, the intended amount of trapped hydrogen may fail to be achieved. If the above hydrogen concentration is more than 35.0% by vol-

## 13

ume, the risk of the steel sheet rupturing in the operation due to hydrogen embrittlement may be increased. Accordingly, the hydrogen concentration in the atmosphere at 730° C. to 950° C. is limited to be 1.0% to 35.0% by volume. As for the lower limit, the above hydrogen concentration is preferably 4.0% by volume or more. As for the upper limit, the above hydrogen concentration is preferably 32.0% by volume or less.

Dew Point at 730° C. to 950° C.: -35° C. to 15° C.

If the dew point at 730° C. to 950° C. is less than -35° C., internal oxidation may fail to occur to a sufficient degree. If the above dew point is more than 15° C., pick-up may be formed and degrade the consistency in the operation. Accordingly, the dew point at 730° C. to 950° C. is limited to be -35° C. to 15° C. As for the lower limit, the above dew point is preferably -30° C. or more. As for the upper limit, the above dew point is preferably 5° C. or less.

Average Cooling Rate Between Annealing Temperature and 600° C.: 5° C./s or More

If the average cooling rate between the annealing temperature and 600° C. is less than 5° C./s, polygonal ferrite may be formed in an excessive amount and, consequently, the microstructure according to aspects of the present invention may fail to be formed. Accordingly, the average cooling rate between the annealing temperature and 600° C. is limited to be 5° C./s or more and is preferably 8° C./s or more. Although the upper limit is not specified, the above average cooling rate is preferably 1500° C./s or less.

Cooling Stop Temperature: More than Ms and 600° C. or Less

If the cooling stop temperature is Ms or less, tempered martensite may be formed, which results in a reduction in TS and the degradation of bendability. If the cooling stop temperature is more than 600° C., polygonal ferrite may be formed in an excessive amount and, consequently, the intended microstructure may fail to be formed. Accordingly, the cooling stop temperature is limited to be more than Ms and 600° C. or less. As for the lower limit, the cooling stop temperature is preferably 440° C. or more. As for the upper limit, the cooling stop temperature is preferably 560° C. or less.

Retention Time at Ms to 600° C.: 1000 s or Less

If the retention time at Ms to 600° C. is more than 1000 s, the ferrite transformation and the bainite transformation may occur to an excessive degree or pearlite may be formed in an excessive amount and, consequently, the intended microstructure may fail to be formed. In addition, the amount of the trapped hydrogen may be reduced and, consequently, the bendability of the steel sheet may become degraded. Accordingly, the retention time at Ms to 600° C. is limited to be 1000 s or less, is preferably 500 s or less, and is more preferably 200 s or less. As for the lower limit, the above retention time is preferably 5 s or more and is more preferably 10 s or more. Optionally, subsequent to a cooling, the temperature may be increased to the intended temperature prior to the retention.

Temperature Range of Ms to 50° C.: 1.0° C./s or More

If the average cooling rate between Ms and 50° C. is less than 1.0° C./s, hydrogen may become dissipated and, consequently, the intended amount of the trapped hydrogen may fail to be achieved. Accordingly, the average cooling rate between Ms and 50° C. is limited to be 1.0° C./s or more. As for the upper limit, the above average cooling rate is preferably 1500° C./s or less. The cooling stop temperature in the cooling step is room temperature. The term "room temperature" used herein refers to a temperature of 15° C. to 25° C.

## 14

Elongation Ratio in Elongation Rolling (Temper Rolling): 0.05% to 1%

If the elongation ratio in elongation rolling is less than 0.05%, the intended amount of the trapped hydrogen may fail to be achieved. If the above elongation ratio is more than 1%, the oxide particles included in the surface layer may become detached. Accordingly, the elongation ratio in elongation rolling is limited to be 0.05% to 1%. As for the lower limit, the above elongation ratio is preferably 0.10% or more. As for the upper limit, the above elongation ratio is preferably 0.7% or less and is more preferably 0.5% or less. Aging Treatment Subsequent to Elongation Rolling:  $(273+T) \times (20+\log_{10}(t)) \geq 6800$ ,  $T \leq 200$ , where T is Temperature (° C.) and t is Time (hr)

When the conditions under which the aging treatment is performed subsequent to the elongation rolling satisfy the above relationship, hydrogen may be trapped by the oxide included in the steel and, consequently, the intended amount of the trapped hydrogen may be achieved. If the above conditions deviate from the relationship, the state in which hydrogen is trapped by the oxide may change and, consequently, the bendability required in accordance with aspects of the present invention may fail to be achieved. Accordingly, the aging treatment performed subsequent to the elongation rolling satisfies  $(273+T) \times (20+\log_{10}(t)) \geq 6800$ ,  $T \leq 200$ , where T is a temperature (° C.) and t is a time (hr).

Although the other conditions for the production method are not limited, for example, the following conditions are preferably employed.

The slab is preferably produced by continuous casting in order to prevent macrosegregation. Ingot casting and thin-slab casting may alternatively be used for preparing the slab. When the slab is hot-rolled, the slab may be cooled to room temperature and subsequently reheated prior to the hot rolling. In another case, the slab may be charged into a heating furnace without being cooled to room temperature before hot rolling. Alternatively, an energy-saving process in which the slab is hot-rolled immediately after heat insulation has been performed simply also be used. When the slab is heated, it is preferable to heat the slab to 1100° C. or more in order to dissolve carbide and prevent an increase in the rolling load. The slab-heating temperature is preferably 1300° C. or less in order to prevent an increase in scale loss.

Note that, the temperature of the slab refers to the temperature of the surface of the slab. Heating rough-rolled steel bars may be performed in hot-rolling of the slab. Alternatively, rough-rolled steel bars joined to one another may be subjected to continuous finish rolling. That is, a "continuous rolling process" may be used. It is preferable to perform, in hot rolling, lubricated rolling with a coefficient of friction of 0.10 to 0.25 in all or a part of the passes of the finish rolling in order to reduce the rolling load and variations in shape and quality of the steel sheet.

Subsequent to the cooling, scale is removed from the steel sheet by pickling or the like. Then, annealing and hot-dip galvanizing are performed. Some of the hot-rolled steel sheets may be cold-rolled prior to annealing.

Optionally, a coating film formation treatment may be performed in any of the steps subsequent to the annealing step. Examples of the coating film formation treatment include a treatment in which roller coating, electrodeposition, immersion, or the like is performed.

In the case where the method for producing the high-strength steel sheet according to aspects of the present invention is a method for producing the high-strength steel sheet that includes a coated layer disposed on the surface,

## 15

the production method according to aspects of the present invention further includes a plating process performed in the cooling step.

The method for the plating process may be a common method appropriate to the coated layer that is to be formed. In the case where a hot-dip galvanizing treatment is performed, an alloying treatment may be performed.

## EXAMPLES

The present invention is specifically described on the basis of Examples below. The scope of the present invention is not limited to Examples below.

Steels having the compositions described in Table 1 (the balance being Fe and inevitable impurities) were prepared in a vacuum melting furnace placed in a laboratory and rolled into steel slabs. The steel slabs were heated to 1200° C. and then rough-rolled. The rough-rolled steel sheets were hot-rolled under the conditions described in Table 2-1 to form hot-rolled steel sheets (HR). Some of the hot-rolled steel sheets were cold-rolled to a thickness of 1.4 mm to form cold-rolled steel sheets (CR). The hot-rolled steel sheets and the cold-rolled steel sheets were annealed. The annealing treatment was performed by heating treatment in a laboratory. For some of the samples, a plating apparatus was further used. The treatment was performed under the conditions described in Tables 2-1 and 2-2. Hereby, cold-rolled steel sheets (CR), hot-dip galvanized steel sheets (GI), and alloyed hot-dip galvanized steel sheets (GA) 1 to 34 were prepared. The hot-dip galvanized steel sheets were prepared by immersing the steel sheets in a plating bath having a temperature of 465° C. to form a coated layer at a coating weight of 35 to 45 g/m<sup>2</sup>. The alloyed galvanized steel sheets were prepared by performing an alloying treatment in which the steel sheets were held at 500° C. to 600° C. for 1 to 60 s subsequent to the formation of the coated layer. Subsequent to the plating process, the temperature was reduced to room temperature at 8° C./s.

The hot-dip galvanized steel sheets and the alloyed hot-dip galvanized steel sheets were subjected to elongation rolling (temper rolling) and an aging treatment and subsequently evaluated in terms of tensile properties and bendability in accordance with the following methods. Table 3 summarizes the results. Table 3 also summarizes the results of observation of the microstructures and the results of observation of the oxides included in the specific regions which were conducted by the above-described methods. In the item regarding the coarse oxide particles, "Absent" is shown when the content of coarse oxide particles having a

## 16

minor axis length of more than 1.0 μm in the region extending 50 μm from the surface of the steel sheet is 1.0×10<sup>8</sup> particles/m<sup>2</sup> or less, while "Present" is shown when the content of coarse oxide particles having a minor axis length of more than 1.0 μm in the region extending 50 μm from the surface of the steel sheet is more than 1.0×10<sup>8</sup> particles/m<sup>2</sup>.

## &lt;Tensile Test&gt;

The TS of each of the annealed steel sheets was measured by taking a JIS No. 5 tensile test specimen (JIS Z 2201) from the annealed steel sheet in a direction perpendicular to the rolling direction and subjecting the specimen to a tensile test conforming to JIS Z 2241 (1998) with a strain rate of 10<sup>-3</sup>/s. In accordance with aspects of the present invention, a sample having a TS of 980 MPa or more was considered acceptable.

## &lt;Bendability&gt;

A strip-shaped test specimen having a width of 30 mm and a length of 100 mm was taken from each of the annealed steel sheets such that the axis about which a bend test was conducted was parallel to the rolling direction. This specimen was subjected to a bend test. Specifically, the test specimen was subjected to a 90°-V bend test with a stroke speed of 50 mm/s, a pressing load of 10 ton, and a press holding time of 5 seconds. The ridge line formed at the vertex of the bent portion was observed with a 10-fold magnifier. The minimum bend radius at which cracks having a length of 0.5 mm or more were not formed was determined. The ratio (R/t) of the minimum bend radius R to the thickness t of the steel sheet was calculated. The ratio (R/t) was used as a measure for the evaluation of bendability.

## &lt;Trapped Hydrogen Content&gt;

A test specimen having a length of 30 mm and a width of 5 mm was taken from each of the annealed steel sheets. After the coated layer had been removed with an alkali, the content of the trapped hydrogen and the peak of desorption of hydrogen were measured. The above measurement was conducted by a thermal desorption method. The heating rate was set to 200° C./hr. Specifically, the temperature was increased from room temperature to 800° C. continuously and then reduced to room temperature. The temperature was again increased to 800° C. at a heating rate of 200° C./hr. The difference between the amount of hydrogen desorbed in the first heating and the amount of hydrogen desorbed in the second heating was considered as the amount of hydrogen desorbed, and part of the desorbed hydrogen which was detected at 350° C. to 600° C. was considered as trapped hydrogen. Table 3 summarizes the results.

TABLE 1

| Steel | Composition (mass%) |      |     |       |        |       |       |                                           | Remark                         |
|-------|---------------------|------|-----|-------|--------|-------|-------|-------------------------------------------|--------------------------------|
|       | C                   | Si   | Mn  | P     | S      | Al    | N     | Others                                    |                                |
| A     | 0.10                | 0.60 | 2.5 | 0.012 | 0.0009 | 0.024 | 0.003 | —                                         | Within the scope of invention  |
| B     | 0.15                | 0.15 | 3.5 | 0.015 | 0.0021 | 0.100 | 0.002 | —                                         | Within the scope of invention  |
| C     | 0.10                | 1.40 | 2.5 | 0.020 | 0.0013 | 0.030 | 0.007 | Mo: 0.15, B: 0.0020                       | Within the scope of invention  |
| D     | 0.15                | 0.40 | 3.5 | 0.025 | 0.0024 | 0.045 | 0.004 | Ti: 0.030, Nb: 0.010, B: 0.0010           | Within the scope of invention  |
| E     | 0.20                | 0.60 | 3.0 | 0.004 | 0.0045 | 0.017 | 0.003 | Cr: 0.50, Nb: 0.030, Mo: 0.10, B: 0.0020  | Within the scope of invention  |
| F     | 0.25                | 1.20 | 2.5 | 0.008 | 0.0005 | 0.029 | 0.005 | Ni: 0.5, Ti: 0.015, Mo: 0.10, REM: 0.0010 | Within the scope of invention  |
| G     | 0.32                | 0.90 | 3.0 | 0.015 | 0.0014 | 0.035 | 0.005 | Mo: 0.20, V: 0.10, Cu: 0.10, Ca: 0.0010   | Within the scope of invention  |
| H     | 0.10                | 0.30 | 3.0 | 0.014 | 0.0022 | 0.015 | 0.003 | Nb: 0.035, Cu: 0.10, B: 0.0020, Sb: 0.010 | Within the scope of invention  |
| I     | 0.37                | 1.80 | 3.5 | 0.013 | 0.0003 | 0.048 | 0.004 | Mo: 0.10, B: 0.0005, Sn: 0.05             | Within the scope of invention  |
| J     | 0.45                | 1.00 | 2.5 | 0.005 | 0.0011 | 0.034 | 0.003 | Ni: 0.30, Ti: 0.015, B: 0.0015, Sn: 0.05  | Outside the scope of invention |
| K     | 0.04                | 0.50 | 3.0 | 0.018 | 0.0006 | 0.036 | 0.005 | Ti: 0.020, Mo: 0.25, B: 0.0020            | Outside the scope of invention |
| L     | 0.15                | 0.05 | 2.5 | 0.015 | 0.0014 | 0.027 | 0.003 | Cr: 0.50, Nb: 0.030, Mo: 0.05, B: 0.0010  | Outside the scope of invention |

TABLE 1-continued

| Steel | Composition (mass%) |      |     |       |        |       |       | Remark                                    |
|-------|---------------------|------|-----|-------|--------|-------|-------|-------------------------------------------|
|       | C                   | Si   | Mn  | P     | S      | Al    | N     |                                           |
| M     | 0.15                | 3.50 | 3.5 | 0.013 | 0.0019 | 0.025 | 0.004 | Ni: 0.50, Ti: 0.020, V: 0.10, B: 0.0020   |
| N     | 0.20                | 0.50 | 1.3 | 0.003 | 0.0030 | 0.036 | 0.005 | Ti: 0.020, Nb: 0.010, Mo: 0.20, B: 0.0020 |
| O     | 0.15                | 1.00 | 4.1 | 0.012 | 0.0024 | 0.030 | 0.003 | Ti: 0.010, Nb: 0.010, Mo: 0.15            |

\*The underlined values are outside the scope of the present invention.

TABLE 2-1

| Steel<br>sheet<br>No | Steel<br>No | Hot rolling                               |                                |                                 |                                           | Cold rolling                      |                       |                                                     |                                       | Annealing                            |                                       |                                   |                       |                     |
|----------------------|-------------|-------------------------------------------|--------------------------------|---------------------------------|-------------------------------------------|-----------------------------------|-----------------------|-----------------------------------------------------|---------------------------------------|--------------------------------------|---------------------------------------|-----------------------------------|-----------------------|---------------------|
|                      |             | Finish<br>rolling<br>temperature<br>(°C.) | Descaling<br>pressure<br>(MPa) | Coiling<br>temperature<br>(°C.) | Cold<br>rolling<br>reduction<br>ratio (%) | Annealing<br>temperature<br>(°C.) | Annealing<br>time (s) | Dew point<br>concentration<br>at 730° C.<br>(vol %) | Average<br>cooling<br>rate<br>(°C./s) | Cooling stop<br>temperature<br>(°C.) | Average<br>heating<br>rate<br>(°C./s) | Retention<br>temperature<br>(°C.) | Retention<br>time (s) | Remark              |
| 1                    | A           | 900                                       | 50                             | 500                             | 50                                        | 810                               | 200                   | -20                                                 | 10                                    | 15                                   | 500                                   | —                                 | 500                   | Invention example   |
| 2                    |             | 980                                       | 50                             | 500                             | 50                                        | 810                               | 200                   | -20                                                 | 10                                    | 15                                   | 500                                   | —                                 | 500                   | Comparative example |
| 3                    |             | 750                                       | 50                             | 500                             | 50                                        | 810                               | 200                   | -20                                                 | 10                                    | 15                                   | 500                                   | —                                 | 500                   | Comparative example |
| 4                    |             | 900                                       | 50                             | 600                             | 50                                        | 810                               | 200                   | -20                                                 | 10                                    | 15                                   | 500                                   | —                                 | 500                   | Comparative example |
| 5                    | B           | 900                                       | 50                             | 500                             | 15                                        | 810                               | 200                   | -20                                                 | 10                                    | 15                                   | 500                                   | —                                 | 500                   | Comparative example |
| 6                    |             | 900                                       | 30                             | 500                             | 50                                        | 900                               | 100                   | -25                                                 | 15                                    | 30                                   | 500                                   | —                                 | 500                   | Invention example   |
| 7                    |             | 900                                       | 30                             | 500                             | 50                                        | 980                               | 100                   | -25                                                 | 15                                    | 30                                   | 500                                   | —                                 | 500                   | Comparative example |
| 8                    |             | 900                                       | 30                             | 500                             | 50                                        | 900                               | 1200                  | -25                                                 | 15                                    | 30                                   | 500                                   | —                                 | 500                   | Comparative example |
| 9                    |             | 900                                       | 30                             | 500                             | 50                                        | 900                               | 1                     | -25                                                 | 15                                    | 30                                   | 500                                   | —                                 | 500                   | Comparative example |
| 10                   |             | 900                                       | 30                             | 500                             | 50                                        | 850                               | 100                   | -25                                                 | 15                                    | 1000                                 | 25                                    | 100                               | 150                   | Invention example   |
| 11                   | C           | 900                                       | 15                             | 450                             | 40                                        | 810                               | 600                   | -35                                                 | 5                                     | 10                                   | 200                                   | 30                                | 400                   | Invention example   |
| 12                   |             | 900                                       | 15                             | 450                             | 40                                        | 700                               | 600                   | -35                                                 | 5                                     | 10                                   | 200                                   | 30                                | 400                   | Comparative example |
| 13                   |             | 900                                       | 15                             | 450                             | 40                                        | 810                               | 600                   | -35                                                 | 5                                     | 4                                    | 200                                   | 30                                | 400                   | Comparative example |
| 14                   |             | 900                                       | 15                             | 450                             | 40                                        | 810                               | 600                   | -35                                                 | 5                                     | 10                                   | 620                                   | —                                 | 620                   | Comparative example |
| 15                   | D           | 900                                       | 30                             | 400                             | —                                         | 830                               | 200                   | -30                                                 | 2                                     | 20                                   | 200                                   | —                                 | 200                   | Invention example   |
| 16                   |             | 900                                       | 30                             | 400                             | —                                         | 830                               | 200                   | -30                                                 | 0.5                                   | 20                                   | 200                                   | —                                 | 200                   | Comparative example |
| 17                   |             | 900                                       | 30                             | 400                             | —                                         | 830                               | 200                   | -40                                                 | 2                                     | 20                                   | 200                                   | —                                 | 200                   | Invention example   |
| 18                   |             | 900                                       | 30                             | 400                             | —                                         | 830                               | 200                   | -30                                                 | 2                                     | 20                                   | 200                                   | —                                 | 200                   | Comparative example |
| 19                   |             | 900                                       | 30                             | 400                             | —                                         | 830                               | 200                   | -30                                                 | 2                                     | 20                                   | 200                                   | —                                 | 200                   | Comparative example |
| 20                   | E           | 850                                       | 30                             | 500                             | 50                                        | 880                               | 200                   | -15                                                 | 20                                    | 50                                   | 460                                   | —                                 | 460                   | Invention example   |
| 21                   |             | 850                                       | 30                             | 500                             | 50                                        | 880                               | 200                   | -15                                                 | 20                                    | 50                                   | 460                                   | —                                 | 460                   | Comparative example |
| 22                   |             | 850                                       | 10                             | 500                             | 50                                        | 880                               | 200                   | -15                                                 | 20                                    | 50                                   | 460                                   | —                                 | 460                   | Comparative example |
| 23                   |             | 850                                       | 30                             | 500                             | 50                                        | 880                               | 200                   | -15                                                 | 20                                    | 50                                   | 460                                   | —                                 | 460                   | Comparative example |
| 24                   |             | 850                                       | 30                             | 500                             | 50                                        | 880                               | 200                   | -15                                                 | 20                                    | 50                                   | 460                                   | —                                 | 460                   | Comparative example |
| 25                   | F           | 900                                       | 30                             | 500                             | 50                                        | 850                               | 200                   | -10                                                 | 25                                    | 15                                   | 550                                   | —                                 | 550                   | Invention example   |
| 26                   | G           | 900                                       | 30                             | 500                             | 50                                        | 750                               | 800                   | -5                                                  | 30                                    | 15                                   | 500                                   | —                                 | 500                   | Comparative example |
| 27                   | H           | 900                                       | 30                             | 500                             | 50                                        | 810                               | 200                   | 0                                                   | 20                                    | 15                                   | 500                                   | —                                 | 500                   | Invention example   |
| 28                   | I           | 900                                       | 30                             | 500                             | 50                                        | 850                               | 200                   | 5                                                   | 25                                    | 15                                   | 500                                   | —                                 | 500                   | Comparative example |
| 29                   | J           | 900                                       | 30                             | 500                             | 50                                        | 810                               | 200                   | 10                                                  | 25                                    | 15                                   | 500                                   | —                                 | 500                   | Invention example   |
| 30                   | K           | 900                                       | 30                             | 500                             | 50                                        | 810                               | 200                   | -5                                                  | 10                                    | 15                                   | 500                                   | —                                 | 500                   | Comparative example |
| 31                   | L           | 900                                       | 30                             | 500                             | 50                                        | 810                               | 200                   | -5                                                  | 10                                    | 15                                   | 500                                   | —                                 | 500                   | Comparative example |
| 32                   | M           | 900                                       | 30                             | 500                             | 50                                        | 890                               | 200                   | -5                                                  | 10                                    | 15                                   | 500                                   | —                                 | 500                   | Comparative example |
| 33                   | N           | 900                                       | 30                             | 500                             | 50                                        | 810                               | 200                   | -5                                                  | 10                                    | 15                                   | 500                                   | —                                 | 500                   | Comparative example |
| 34                   | O           | 900                                       | 30                             | 500                             | 50                                        | 810                               | 200                   | -5                                                  | 10                                    | 15                                   | 500                                   | —                                 | 500                   | Comparative example |

TABLE 2-2

| Steel<br>sheet<br>No. | Galvanization                         |                                   |                                 | Average<br>cooling rate              |                         |                                |      | Aging<br>time<br>(hr) | Formula<br>(1) | *Surface<br>condition | Remark |
|-----------------------|---------------------------------------|-----------------------------------|---------------------------------|--------------------------------------|-------------------------|--------------------------------|------|-----------------------|----------------|-----------------------|--------|
|                       | Plating bath<br>temperature<br>(° C.) | Alloying<br>temperature<br>(° C.) | Alloying<br>holding<br>time (s) | between Ms<br>and 50° C.<br>(° C./s) | Elongation<br>ratio (%) | Aging<br>temperature<br>(° C.) |      |                       |                |                       |        |
| 1                     | —                                     | —                                 | —                               | 20                                   | 0.3                     | 25                             | 1200 | 6878                  | CR             | Invention example     |        |
| 2                     | —                                     | —                                 | —                               | 20                                   | 0.3                     | 25                             | 1200 | 6878                  | CR             | Comparative example   |        |
| 3                     | —                                     | —                                 | —                               | 20                                   | 0.3                     | 25                             | 1200 | 6878                  | CR             | Comparative example   |        |
| 4                     | —                                     | —                                 | —                               | 20                                   | 0.3                     | 25                             | 1200 | 6878                  | CR             | Comparative example   |        |
| 5                     | —                                     | —                                 | —                               | 20                                   | 0.3                     | 25                             | 1200 | 6878                  | CR             | Comparative example   |        |
| 6                     | 465                                   | —                                 | —                               | 50                                   | 0.6                     | 100                            | 240  | 8348                  | GI             | Invention example     |        |
| 7                     | 465                                   | —                                 | —                               | 50                                   | 0.6                     | 100                            | 240  | 8348                  | GI             | Comparative example   |        |
| 8                     | 465                                   | —                                 | —                               | 50                                   | 0.6                     | 100                            | 240  | 8348                  | GI             | Comparative example   |        |
| 9                     | 465                                   | —                                 | —                               | 50                                   | 0.6                     | 100                            | 240  | 8348                  | GI             | Comparative example   |        |
| 10                    | —                                     | —                                 | —                               | 1000                                 | 0.6                     | 100                            | 240  | 8348                  | CR             | Invention example     |        |
| 11                    | —                                     | —                                 | —                               | 5                                    | 0.3                     | 50                             | 720  | 7383                  | CR             | Invention example     |        |
| 12                    | —                                     | —                                 | —                               | 5                                    | 0.3                     | 50                             | 720  | 7383                  | CR             | Comparative example   |        |
| 13                    | —                                     | —                                 | —                               | 5                                    | 0.3                     | 50                             | 720  | 7383                  | CR             | Comparative example   |        |
| 14                    | —                                     | —                                 | —                               | 5                                    | 0.3                     | 50                             | 720  | 7383                  | CR             | Comparative example   |        |
| 15                    | 465                                   | 520                               | 20                              | 20                                   | 0.3                     | 75                             | 120  | 7684                  | GA             | Invention example     |        |
| 16                    | 465                                   | 520                               | 20                              | 20                                   | 0.3                     | 75                             | 120  | 7684                  | GA             | Comparative example   |        |
| 17                    | 465                                   | 520                               | 20                              | 20                                   | 0.3                     | 75                             | 120  | 7684                  | GA             | Comparative example   |        |
| 18                    | 465                                   | 520                               | 20                              | 20                                   | 0                       | 75                             | 120  | 7684                  | GA             | Comparative example   |        |
| 19                    | 465                                   | 520                               | 20                              | 20                                   | 0.3                     | 75                             | 120  | 7684                  | GA             | Comparative example   |        |
| 20                    | 465                                   | 520                               | 20                              | 10                                   | 0.6                     | 50                             | 1200 | 7455                  | GA             | Invention example     |        |
| 21                    | 465                                   | 520                               | 20                              | —0.5                                 | 0.6                     | 50                             | 1200 | 7455                  | GA             | Comparative example   |        |
| 22                    | 465                                   | 520                               | 20                              | 10                                   | 0.6                     | 50                             | 1200 | 7455                  | GA             | Comparative example   |        |
| 23                    | 465                                   | 520                               | 20                              | 10                                   | 0.6                     | 250                            | 1    | 10460                 | GA             | Comparative example   |        |
| 24                    | 465                                   | 520                               | 20                              | 10                                   | 0.6                     | 25                             | 480  | 6759                  | GA             | Comparative example   |        |
| 25                    | 465                                   | —                                 | —                               | 20                                   | 0.1                     | 180                            | 0.1  | 8607                  | GI             | Invention example     |        |
| 26                    | 465                                   | 520                               | 20                              | 20                                   | 0.1                     | 200                            | 1    | 9460                  | GA             | Invention example     |        |
| 27                    | 465                                   | 520                               | 20                              | 20                                   | 1.0                     | 25                             | 1200 | 6878                  | GA             | Invention example     |        |
| 28                    | 465                                   | 560                               | 20                              | 20                                   | 0.3                     | 200                            | 10   | 9933                  | GA             | Invention example     |        |
| 29                    | 465                                   | 520                               | 20                              | 20                                   | 0.3                     | 25                             | 2160 | 6954                  | GA             | Comparative example   |        |
| 30                    | 465                                   | 520                               | 20                              | 20                                   | 0.3                     | 25                             | 1440 | 6901                  | GA             | Comparative example   |        |
| 31                    | 465                                   | 520                               | 20                              | 20                                   | 0.3                     | 25                             | 1440 | 6901                  | GA             | Comparative example   |        |
| 32                    | 465                                   | 580                               | 20                              | 20                                   | 0.3                     | 25                             | 1440 | 6901                  | GA             | Comparative example   |        |
| 33                    | 465                                   | 520                               | 20                              | 20                                   | 0.3                     | 25                             | 1440 | 6901                  | GA             | Comparative example   |        |
| 34                    | 465                                   | 520                               | 20                              | 20                                   | 0.3                     | 25                             | 1440 | 6901                  | GA             | Comparative example   |        |

\*Surface condition CR: Cold-rolled steel sheet, GI: Hot-dip galvanized steel sheet, GA: Alloyed hot dip galvanized steel sheet

\*The underlined values are outside the scope of the present invention.

TABLE 3

| Steel<br>sheet<br>No. | *Microstructure |             |             |                       |             |              |              | Content of<br>hydrogen<br>trapped in                   |                                 |          |      | Mechanical<br>properties<br>Remark |                     |
|-----------------------|-----------------|-------------|-------------|-----------------------|-------------|--------------|--------------|--------------------------------------------------------|---------------------------------|----------|------|------------------------------------|---------------------|
|                       | V(H)<br>(%)     | V(M)<br>(%) | V(γ)<br>(%) | Others<br>V(P)<br>(%) | V(S)<br>(%) | V(Fs)<br>(%) | D(M)<br>(μm) | *1 (10 <sup>10</sup><br>Particles/<br>m <sup>2</sup> ) | steel sheet<br>(ppm by<br>mass) | TS (MPa) | R/t  |                                    |                     |
| 1                     | 49              | 38          | 2           | 0                     | 51          | 0            | 2            | 56                                                     | Absent                          | 0.31     | 1000 | 0.4                                | Invention example   |
| 2                     | 52              | 38          | 3           | 0                     | 48          | 0            | 22           | 53                                                     | Absent                          | 0.30     | 992  | 2.5                                | Comparative example |
| 3                     | 50              | 39          | 1           | 0                     | 50          | 3            | 3            | 53                                                     | Absent                          | 0.33     | 1007 | 2.1                                | Comparative example |
| 4                     | 44              | 36          | 2           | 0                     | 56          | 0            | 8            | 92                                                     | Present                         | 0.36     | 988  | 2.1                                | Comparative example |
| 5                     | 52              | 38          | 1           | 0                     | 48          | 7            | 3            | 50                                                     | Absent                          | 0.31     | 1039 | 2.5                                | Comparative example |
| 6                     | 100             | 96          | 4           | 0                     | 0           | 0            | 16           | 13                                                     | Absent                          | 0.11     | 1394 | 3.2                                | Invention example   |
| 7                     | 100             | 96          | 4           | 0                     | 0           | 0            | 28           | 10                                                     | Absent                          | 0.09     | 1330 | 4.3                                | Comparative example |
| 8                     | 100             | 97          | 3           | 0                     | 0           | 0            | 21           | 14                                                     | Absent                          | 0.12     | 1384 | 3.6                                | Comparative example |
| 9                     | 82              | 82          | 0           | 0                     | 18          | 0            | 11           | 12                                                     | Absent                          | 0.02     | 1388 | 4.3                                | Comparative example |
| 10                    | 100             | 99          | 1           | 0                     | 0           | 0            | 11           | 11                                                     | Absent                          | 0.10     | 1390 | 2.9                                | Invention example   |
| 11                    | 52              | 3           | 3           | 0                     | 48          | 0            | 1            | 150                                                    | Absent                          | 0.49     | 1031 | 1.1                                | Invention example   |
| 12                    | 17              | 15          | 1           | 0                     | 83          | 0            | 1            | 140                                                    | Absent                          | 0.46     | 858  | 0.4                                | Comparative example |
| 13                    | 27              | 26          | 1           | 0                     | 73          | 0            | 1            | 150                                                    | Absent                          | 0.48     | 946  | 0.4                                | Comparative example |
| 14                    | 26              | 25          | 1           | 3                     | 71          | 0            | 5            | 180                                                    | Absent                          | 0.50     | 963  | 0.7                                | Comparative example |
| 15                    | 97              | 93          | 4           | 0                     | 3           | 0            | 6            | 72                                                     | Absent                          | 0.35     | 1365 | 2.9                                | Invention example   |
| 16                    | 98              | 93          | 5           | 0                     | 2           | 0            | 5            | 70                                                     | Absent                          | 0.03     | 1374 | 3.6                                | Comparative example |
| 17                    | 97              | 92          | 5           | 0                     | 3           | 0            | 5            | 0.7                                                    | Absent                          | 0.03     | 1360 | 3.6                                | Comparative example |
| 18                    | 97              | 92          | 5           | 0                     | 3           | 0            | 5            | 73                                                     | Absent                          | 0.02     | 1368 | 3.6                                | Comparative example |
| 19                    | 97              | 93          | 4           | 0                     | 3           | 0            | 6            | 70                                                     | Absent                          | 0.02     | 1357 | 3.9                                | Comparative example |
| 20                    | 100             | 95          | 5           | 0                     | 0           | 0            | 7            | 100                                                    | Absent                          | 0.37     | 1568 | 3.2                                | Invention example   |
| 21                    | 100             | 82          | 10          | 0                     | 0           | 0            | 8            | 110                                                    | Absent                          | 0.04     | 1523 | 4.3                                | Comparative example |

TABLE 3-continued

| Steel sheet | *Microstructure |      |               |        |     |      |       |            | *1 ( $10^{10}$ Particles/<br>m <sup>2</sup> ) | Content of<br>hydrogen<br>trapped in<br>steel sheet<br>(ppm by<br>mass) | Mechanical<br>properties |     |                     |
|-------------|-----------------|------|---------------|--------|-----|------|-------|------------|-----------------------------------------------|-------------------------------------------------------------------------|--------------------------|-----|---------------------|
|             | V(H)            | V(M) | V( $\gamma$ ) | Others |     | V(S) | V(Fs) | D(M)       |                                               |                                                                         | TS (MPa)                 | R/t | Remark              |
|             | No.             | (%)  | (%)           | (%)    | (%) | (%)  | (%)   | ( $\mu$ m) |                                               |                                                                         |                          |     |                     |
| 22          | 100             | 94   | 6             | 0      | 0   | 0    | 7     | 110        | Present                                       | 0.15                                                                    | 1562                     | 3.9 | Comparative example |
| 23          | 99              | 96   | 3             | 1      | 0   | 0    | 8     | 96         | Absent                                        | 0.03                                                                    | 1488                     | 4.3 | Comparative example |
| 24          | 100             | 95   | 5             | 0      | 0   | 0    | 7     | 110        | Absent                                        | 0.04                                                                    | 1564                     | 4.3 | Comparative example |
| 25          | 100             | 93   | 7             | 0      | 0   | 0    | 11    | 130        | Absent                                        | 0.50                                                                    | 1695                     | 3.2 | Invention example   |
| 26          | 92              | 80   | 12            | 0      | 8   | 0    | 12    | 100        | Absent                                        | 0.45                                                                    | 1924                     | 4.3 | Invention example   |
| 27          | 91              | 85   | 3             | 0      | 9   | 0    | 8     | 45         | Absent                                        | 0.22                                                                    | 1078                     | 1.4 | Invention example   |
| 28          | 100             | 87   | 13            | 0      | 0   | 0    | 13    | 120        | Absent                                        | 0.61                                                                    | 2081                     | 5.0 | Invention example   |
| 29          | 97              | 79   | 15            | 0      | 3   | 0    | 15    | 90         | Absent                                        | 0.41                                                                    | 2220                     | 7.1 | Comparative example |
| 30          | 65              | 45   | 4             | 0      | 35  | 0    | 4     | 85         | Absent                                        | 0.34                                                                    | 883                      | 0.2 | Comparative example |
| 31          | 97              | 92   | 1             | 0      | 3   | 0    | 7     | —0.7       | Absent                                        | 0.03                                                                    | 1326                     | 3.9 | Comparative example |
| 32          | 100             | 93   | 7             | 0      | 0   | 0    | 7     | 410        | Absent                                        | 0.74                                                                    | 1544                     | 4.6 | Comparative example |
| 33          | 37              | 14   | 5             | 0      | 63  | 0    | 4     | 95         | Absent                                        | 0.38                                                                    | 912                      | 2.5 | Comparative example |
| 34          | 100             | 92   | 8             | 0      | 0   | 0    | 5     | 120        | Absent                                        | 0.53                                                                    | 1539                     | 4.6 | Comparative example |

\*V(H): total area fraction of lower bainite, martensite, and retained austenite, V(M): area fraction of martensite, V( $\gamma$ ): area fraction of retained austenite, V(P): area fraction of pearlite, V(S): total area fraction of upper bainite and ferrite, V(Fs): area fraction of elongated ferrite phase grains having an aspect ratio of 3 or more, D(M): average crystal grain size of martensite included in a region extending 50  $\mu$ m from a surface of the steel sheet

\*1: oxide particles having a minor axis length of 0.8  $\mu$ m or less in the region extending 50  $\mu$ m from the surface of the steel sheet,

\*2: coarse oxide particles having a minor axis length of more than 1.0  $\mu$ m in the region extending 50  $\mu$ m from the surface of the steel sheet

\*The underlined values are outside the scope of the present invention.

In Invention examples, the ratio R/t was 1.5 or less when the TS was 980 MPa or more and less than 1180 MPa, 2.5 or less when the TS was 1180 MPa or more and less than 1320 MPa, 3.5 or less when the TS was 1320 MPa or more and less than 1600 MPa, and 5.0 or less when the TS was 1600 MPa or more and less than 2100 MPa. In contrast, in Comparative examples, which were outside the scope of the present invention, any of the intended TS and the intended bendability failed to be achieved.

#### INDUSTRIAL APPLICABILITY

Using the high-strength steel sheet according to aspects of the present invention for producing automotive components may markedly improve the collision safety and the fuel economy of automobiles.

The invention claimed is:

1. A high-strength steel sheet having a tensile strength of 980 MPa or more comprising:

a composition containing, by mass,

C: 0.05% to 0.40%,

Si: 0.10% to 3.0%,

Mn: 1.5% to 4.0%,

P: 0.100% or less excluding 0%,

S: 0.02% or less excluding 0%,

Al: 0.010% to 1.0%,

N: 0.010% or less,

with the balance being Fe and inevitable impurities;

a microstructure including lower bainite, martensite, retained austenite, upper bainite, and ferrite wherein, a total area fraction of the lower bainite, the martensite, and the retained austenite is 40% to 100%, an area fraction of the retained austenite is 15% or less, and a total area fraction of the upper bainite and the ferrite is 0% to 60%,

wherein, in the microstructure, an area fraction of elongated ferrite phase grains having an aspect ratio of 3 or more is 1% or less, an average crystal grain size of martensite included in a region extending 50  $\mu$ m from a surface of the steel sheet is 20  $\mu$ m or less, a content of oxide particles having a minor axis length of 0.8  $\mu$ m

or less in the region extending 50  $\mu$ m from the surface of the steel sheet is  $1.0 \times 10^{10}$  particles/m<sup>2</sup> or more, and a content of coarse oxide particles having a minor axis length of more than 1.0  $\mu$ m in the region extending 50  $\mu$ m from the surface of the steel sheet is  $1.0 \times 10^8$  particles/m<sup>2</sup> or less; and a content of trapped hydrogen in the steel sheet is 0.05 ppm by mass or more.

2. The high-strength steel sheet according to claim 1, further comprising one or more elements selected from, by mass:

Cr: 0.005% to 2.0%,

Ti: 0.005% to 0.20%,

Nb: 0.005% to 0.20%,

Mo: 0.005% to 2.0%,

V: 0.005% to 2.0%,

Ni: 0.005% to 2.0%,

Cu: 0.005% to 2.0%,

B: 0.0001% to 0.0050%,

Ca: 0.0001% to 0.0050%,

REM: 0.0001% to 0.0050%,

Sn: 0.01% to 0.50%, and

Sb: 0.0010% to 0.10%.

3. The high-strength steel sheet according to claim 1, comprising a coating film constituted by one or more layers, the coating film being disposed on the surface of the steel sheet.

4. The high-strength steel sheet according to claim 1, comprising a galvanizing layer disposed on the surface of the steel sheet.

5. The high-strength steel sheet according to claim 1, comprising an alloyed hot-dip galvanizing layer disposed on the surface of the steel sheet.

6. The high-strength steel sheet according to claim 2, comprising a coating film constituted by one or more layers, the coating film being disposed on the surface of the steel sheet.

7. The high-strength steel sheet according to claim 2, comprising a galvanizing layer disposed on the surface of the steel sheet.

## 25

8. The high-strength steel sheet according to claim 2, comprising an alloyed hot-dip galvanizing layer disposed on the surface of the steel sheet.

9. A method for producing the high-strength steel sheet according to claim 1, the method comprising:

a hot-rolling step of rough-rolling a slab having the composition according to claim 1, subsequently performing descaling at a pressure of 15 MPa or more, then performing finish rolling at 800° C. to 950° C., performing cooling subsequent to the finish rolling, and then performing coiling at 550° C. or less;

10 an annealing step of heating a hot-rolled steel sheet produced in the hot-rolling step to 730° C. to 950° C. and performing holding at 730° C. to 950° C. in an atmosphere having a hydrogen concentration of 1.0% to 35.0% by volume and a dew point of -35° C. to 15° C. for 10 to 1000 s;

15 a cooling step of cooling a steel sheet treated in the annealing step to 600° C. at an average rate of 5° C./s or more, stopping the cooling at a temperature of more than Ms and 600° C. or less, subsequently performing retention at a temperature of more than Ms and 600° C. or less for 1000 s or less, and, subsequent to the retention, performing cooling to room temperature such that the average cooling rate between Ms and 50° C. is 20 1.0° C./s or more;

25 an elongation rolling step of rolling a steel sheet treated in the cooling step at an elongation ratio of 0.05% to 1%; and

30 an aging treatment step of subjecting a steel sheet treated in the elongation rolling step to an aging treatment under conditions satisfying Formula (1) below,

$$(273+T) \times (20 + \log_{10}(t)) \geq 6800, \quad (1)$$

35 wherein in Formula (1), T is an aging temperature in ° C. of 200° C. or less, and t is an aging time in hr.

10 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 10120 10125 10130 10135 10140 10145 10150 10155 10160 10165 10170 10175 10180 10185 10190 10195 10200 10205 10210 10215 10220 10225 10230 10235 10240 10245 10250 10255 10260 10265 10270 10275 10280 10285 10290 10295 10300 10305 10310 10315 10320 10325 10330 10335 10340 10345 10350 10355 10360 10365 10370 10375 10380 10385 10390 10395 10400 10405 10410 10415 10420 10425 10430 10435 10440 10445 10450 10455 10460 10465 10470 10475 10480 10485 10490 10495 10500 10505 10510 10515 10520 10525 10530 10535 10540 10545 10550 10555 10560 10565 10570 10575 10580 10585 10590

27

an elongation rolling step of rolling a steel sheet treated in the cooling step at an elongation ratio of 0.05% to 1%; and

an aging treatment step of subjecting a steel sheet treated in the elongation rolling step to an aging treatment under conditions satisfying Formula (1) below,

$$(273+T) \times (20 + \log_{10}(t)) \geq 6800, \quad (1)$$

wherein in Formula (1), T is an aging temperature in °C. of 100° C. or less, and t is an aging time in hr.

13. The method for producing a high-strength steel sheet according to claim 9, wherein a coating film formation treatment is performed in any of the steps subsequent to the annealing step.

14. The method for producing a high-strength steel sheet according to claim 9, wherein a galvanizing treatment is performed in the cooling step.

15. The method for producing a high-strength steel sheet according to claim 10, wherein a coating film formation treatment is performed in any of the steps subsequent to the annealing step.

16. The method for producing a high-strength steel sheet according to claim 10, wherein a galvanizing treatment is 25 performed in the cooling step.

28

17. The method for producing a high-strength steel sheet according to claim 11, wherein a coating film formation treatment is performed in any of the steps subsequent to the annealing step.

18. The method for producing a high-strength steel sheet according to claim 11, wherein a galvanizing treatment is performed in the cooling step.

19. The method for producing a high-strength steel sheet according to claim 12, wherein a coating film formation treatment is performed in any of the steps subsequent to the annealing step.

20. The method for producing a high-strength steel sheet according to claim 12, wherein a galvanizing treatment is performed in the cooling step.

21. The method for producing a high-strength steel sheet according to claim 14, wherein an alloying treatment is further performed subsequent to the galvanizing treatment.

22. The method for producing a high-strength steel sheet according to claim 16, wherein an alloying treatment is further performed subsequent to the galvanizing treatment.

23. The method for producing a high-strength steel sheet according to claim 18, wherein an alloying treatment is further performed subsequent to the galvanizing treatment.

24. The method for producing a high-strength steel sheet according to claim 20, wherein an alloying treatment is further performed subsequent to the galvanizing treatment.

\* \* \* \* \*